

No. 888,864.

PATENTED MAY 26, 1908.

B. N. BEARD.

ROAD AND PROCESS OF MAKING SAME.

APPLICATION FILED JAN. 29, 1908.



Witnesses:

H. A. Lamb,  
S. W. Atherton.

Inventor  
Bennett N. Beard  
By Attorney  
A. M. Worcester

# UNITED STATES PATENT OFFICE.

BENNETT N. BEARD, OF SHELTON, CONNECTICUT.

## ROAD AND PROCESS OF MAKING SAME.

No. 888,864.

Specification of Letters Patent.

Patented May 26, 1908.

Application filed January 29, 1908. Serial No. 413,271.

*To all whom it may concern:*

Be it known that I, BENNETT N. BEARD, a citizen of the United States, residing at Shelton, county of Fairfield, State of Connecticut, have invented a new and useful 5 Road and Process of Making Same, of which the following is a specification.

This invention relates to the making of the class of roads known generically as macadam roads; that is, roads having an upper stratum 10 of small broken stone or gravel lying upon either a soft or hard sub-stratum.

I have found in practice that an inexpensive, smooth and relatively durable road may 15 be produced by placing an upper stratum of small broken stone or gravel upon any suitable sub-stratum, top dressing with sand to fill the voids and then grouting with a thin mixture of water and cement held in mechanical 20 suspension and sprinkled upon the surface, the water causing the cement to fill the interstices of the upper layer and the setting of the cement producing a hard, firm and very durable surface. And I have found 25 that an exceedingly durable high-grade road may be made by first laying a sub-stratum of relatively large stones with the voids filled with sand and placing thereon an upper stratum consisting of gravel or relatively 30 small broken stone, top dressing with sand and grouting as before.

It is of course well understood that cement if allowed to set properly makes a very hard and durable road bed, but that as cement is 35 ordinarily used, that is mixed with broken stone or gravel and then spread upon the road bed and rolled, it becomes partially set before the spreading and rolling operations are completed and the hardness and durability 40 of the road bed is seriously impaired; in other words, in order to secure the best results from the use of cement in road making it is necessary that the cement be placed on the road bed immediately after mixing 45 and that the road bed remain undisturbed until the cement is set. This can only be effected by mixing the cement as it is used and allowing it to remain undisturbed on the road bed.

50 The object of the present invention is to produce an inexpensive, smooth, hard and durable surface for either top dressed roads, so called, or for deeply laid macadam or Tel-fool roads; in other words, to produce an 55 inexpensive, smooth and hard surface for

either well-laid or relatively inexpensive roads.

The drawing is a cross section illustrating the application of my invention to the making of a high grade road.

10 denotes a substratum of relatively large stones, 11 sand in the voids between the stones, 12 an upper layer of relatively small stones or gravel, 13 a top dressing of sand and 14 a grouting of water and cement in 15 mechanical suspension which is sprinkled upon the surface.

In carrying out my novel process as applied to top-dressed roads, the road is first made smooth and rolled in the ordinary 20 or any preferred manner, then a layer of broken stone or gravel is placed thereon, then a top dressing of sand which is rolled into the broken stone or gravel to fill the voids and the road is grouted by sprinkling 25 the surface with a thin mixture of water and cement held in mechanical suspension, so that there can be no setting of the cement until it is delivered upon the surface of the road, the water causing the cement to fill the 30 interstices in the upper stratum and the mode of placing the cement upon the road permitting it to set undisturbed, thereby producing the best possible results in the 35 least expensive manner.

When it is desired to apply my novel process to the making of high grade roads, a substratum is made of relatively large stones with the voids filled with sand. An upper 40 layer of gravel or small broken stone is then placed thereon, which is top-dressed with sand and the road thus prepared is grouted by sprinkling the surface with a thin mixture of water and cement held in mechanical 45 suspension.

A very firm and durable foundation upon which to lay an asphalt, brick or wooden block pavement may be formed in substantially the same manner, the preparation of the sub-stratum not being an essential part 50 of the invention, the essential feature of which is the grouting of the upper stratum with a thin mixture of water and cement held in mechanical 55 suspension. I have found in practice that my novel process, owing to the fact that the cement is allowed to set under the best conditions possible, produces a smooth and water-tight surface for either a pavement foundation or a road, that has an inherent durability far in excess of 60

any type of surface heretofore produced and which when applied to a well-laid foundation produces a roadway that is practically indestructible for a long time.

5 Having thus described my invention I claim:

1. The process of making roads, which consists in preparing a sub-stratum, then placing thereon an upper stratum of relatively small stones, then top-dressing the same with sand and then sprinkling with a thin mixture of water and cement held in mechanical suspension.

10 2. The process of making roads, which consists in laying a sub-stratum of relatively large stones, filling the voids with sand, then laying an upper stratum of relatively small stones, placing thereon a top dressing of sand and then grouting with a thin mixture of

water and cement held in mechanical suspension and delivered upon the surface.

20 3. A road, consisting of a sub-stratum, an upper stratum of relatively small stones, a top dressing of sand and a grouting of water and cement held in mechanical suspension.

25 4. A road, consisting of a sub-stratum of relatively large stones, a dressing of sand for filling the voids, an upper layer of relatively small stones, a top dressing of sand and a grouting of water and cement held in me- 30 chanical suspension.

In testimony whereof I affix my signature, in presence of two witnesses.

BENNETT N. BEARD.

Witnesses:

A. M. WOOSTER,  
S. W. ATHERTON.